



US008353974B2

(12) **United States Patent**  
**Cooley et al.**

(10) **Patent No.:** **US 8,353,974 B2**  
(45) **Date of Patent:** **\*Jan. 15, 2013**

(54) **SUPERABRASIVE ELEMENTS, METHODS OF MANUFACTURING, AND DRILL BITS INCLUDING SAME**

(75) Inventors: **Craig H. Cooley**, Saratoga Springs, UT (US); **Kenneth E. Bertagnolli**, Riverton, UT (US); **Michael A. Vail**, Genola, UT (US)

(73) Assignee: **US Synthetic Corporation**, Orem, UT (US)

(\*) Notice: Subject to any disclaimer, the term of this patent is extended or adjusted under 35 U.S.C. 154(b) by 0 days.

This patent is subject to a terminal disclaimer.

(21) Appl. No.: **13/478,530**

(22) Filed: **May 23, 2012**

(65) **Prior Publication Data**

US 2012/0228037 A1 Sep. 13, 2012

**Related U.S. Application Data**

(63) Continuation of application No. 11/899,691, filed on Sep. 7, 2007, now Pat. No. 8,202,335.

(60) Provisional application No. 60/850,969, filed on Oct. 10, 2006.

(51) **Int. Cl.**

|                   |           |
|-------------------|-----------|
| <b>B21K 5/02</b>  | (2006.01) |
| <b>B21K 5/04</b>  | (2006.01) |
| <b>B24D 18/00</b> | (2006.01) |
| <b>B24D 3/00</b>  | (2006.01) |
| <b>B24D 3/02</b>  | (2006.01) |
| <b>B24D 3/04</b>  | (2006.01) |
| <b>E21B 10/36</b> | (2006.01) |
| <b>E21B 10/46</b> | (2006.01) |

(52) **U.S. Cl.** ..... **51/307; 51/293; 51/295; 76/108.2; 175/426; 175/434; 175/435**

(58) **Field of Classification Search** ..... None  
See application file for complete search history.

(56) **References Cited**

**U.S. PATENT DOCUMENTS**

|             |         |                     |
|-------------|---------|---------------------|
| 3,745,623 A | 7/1973  | Wentorf, Jr. et al. |
| 4,224,380 A | 9/1980  | Bovenkerk et al.    |
| 4,268,276 A | 5/1981  | Bovenkerk           |
| 4,333,902 A | 6/1982  | Hara                |
| 4,410,054 A | 10/1983 | Nagel et al.        |
| 4,468,138 A | 8/1984  | Nagel               |
| 4,560,014 A | 12/1985 | Geczy               |
| 4,738,322 A | 4/1988  | Hall et al.         |
| 4,811,801 A | 3/1989  | Salesky et al.      |
| 4,913,247 A | 4/1990  | Jones               |
| 5,016,718 A | 5/1991  | Tandberg            |

(Continued)

**FOREIGN PATENT DOCUMENTS**

EP 0352811 1/1990  
(Continued)

**OTHER PUBLICATIONS**

U.S. Appl. No. 60/850,969, filed Oct. 10, 2006, Cooley, et al.

(Continued)

*Primary Examiner* — Melvin C Mayes

*Assistant Examiner* — Colin W Slifka

(74) *Attorney, Agent, or Firm* — Workman Nydegger

(57) **ABSTRACT**

Methods of manufacturing a superabrasive element and/or compact are disclosed. In one embodiment, a superabrasive volume including a tungsten carbide layer may be formed. Polycrystalline diamond elements and/or compacts are disclosed. Rotary drill bits for drilling a subterranean formation and including at least one superabrasive element and/or compact are also disclosed.

**24 Claims, 10 Drawing Sheets**



# US 8,353,974 B2

Page 2

---

## U.S. PATENT DOCUMENTS

|              |         |                    |
|--------------|---------|--------------------|
| 5,092,687 A  | 3/1992  | Hall               |
| 5,120,327 A  | 6/1992  | Dennis             |
| 5,135,061 A  | 8/1992  | Newton, Jr.        |
| 5,154,245 A  | 10/1992 | Waldenstrom et al. |
| 5,364,192 A  | 11/1994 | Damm et al.        |
| 5,368,398 A  | 11/1994 | Damm et al.        |
| 5,370,944 A  | 12/1994 | Omori et al.       |
| 5,460,233 A  | 10/1995 | Meany et al.       |
| 5,480,233 A  | 1/1996  | Cunningham         |
| 5,544,713 A  | 8/1996  | Dennis             |
| 5,952,102 A  | 9/1999  | Cutler             |
| 6,524,357 B2 | 2/2003  | Baldoni et al.     |
| 6,793,861 B2 | 9/2004  | McBain et al.      |
| 6,800,383 B1 | 10/2004 | Lakhotkin et al.   |
| 6,890,655 B2 | 5/2005  | Liu et al.         |
| 7,022,403 B1 | 4/2006  | Lakhotkin et al.   |
| 7,060,641 B2 | 6/2006  | Quian et al.       |
| 7,166,371 B2 | 1/2007  | Lakhotkin et al.   |
| 7,604,073 B2 | 10/2009 | Cooley et al.      |

|                 |         |                   |
|-----------------|---------|-------------------|
| 2006/0157286 A1 | 7/2006  | Pope              |
| 2006/0266558 A1 | 11/2006 | Middlemiss et al. |
| 2008/0085407 A1 | 4/2008  | Cooley et al.     |

## FOREIGN PATENT DOCUMENTS

|    |                |         |
|----|----------------|---------|
| GB | 2362655        | 11/2001 |
| WO | WO 2008/097284 | 8/2008  |

## OTHER PUBLICATIONS

U.S. Appl. No. 10/654,512, filed Sep. 3, 2010, Hall.  
U.S. Appl. No. 11/545,929, filed Oct. 10, 2006, Bertagnolli, et al.  
International Search Report and Written Opinion from PCT International Application No. PCT/US2007/021464 mailed Oct. 28, 2008.  
U.S. Appl. No. 11/899,691, Mail Date Aug. 5, 2010, Office Action.  
U.S. Appl. No. 11/899,691, Mail Date Mar. 2, 2011, Office Action.  
U.S. Appl. No. 11/899,691, Mail Date May 18, 2011, Office Action.  
U.S. Appl. No. 11/899,691, Mail Date Jan. 5, 2012, Office Action.  
U.S. Appl. No. 11/899,691, Mail Date Mar. 7, 2012, Notice of Allowance.



**FIG. 1A**



**FIG. 1B**



**FIG. 2A**



**FIG. 2B**



**FIG. 3**

**FIG. 4****FIG. 5**

**FIG. 6****FIG. 7**

**FIG. 8****FIG. 9**

**FIG. 10****FIG. 11**

**FIG. 12**

**FIG. 13**

**FIG. 14A****FIG. 14B**



**FIG. 15**

**SUPERABRASIVE ELEMENTS, METHODS  
OF MANUFACTURING, AND DRILL BITS  
INCLUDING SAME**

**CROSS-REFERENCE TO RELATED  
APPLICATIONS**

This application is a continuation of U.S. application Ser. No. 11/899,691 filed on 7 Sep. 2007 (now U.S. Pat. No. 8,202,335 issued on 19 Jun. 2012), which claims priority to U.S. Provisional Application Ser. No. 60/850,969 filed on 10 Oct. 2006, each of which is incorporated herein, in its entirety, by this reference.

**BACKGROUND**

Wear-resistant compacts comprising superabrasive (i.e., superhard) material are utilized for a variety of applications and in a corresponding variety of mechanical systems. For example, wear resistant superabrasive elements are used in drilling tools (e.g., inserts, cutting elements, gage trimmers, etc.), machining equipment, bearing apparatuses, wire drawing machinery, and in other mechanical systems.

In one particular example, polycrystalline diamond compacts have found particular utility as cutting elements in drill bits (e.g., roller cone drill bits and fixed cutter drill bits) and as bearing surfaces in so-called "thrust-bearing" apparatuses. A polycrystalline diamond compact ("PDC") cutting element or cutter typically includes a diamond layer or table formed by a sintering process employing high-temperature and high-pressure conditions that causes the diamond table to become bonded to a substrate (e.g., a cemented tungsten carbide substrate), as described in greater detail below.

When a polycrystalline diamond compact is used as a cutting element, it may be mounted to a drill bit either by press-fitting, brazing, or otherwise coupling the cutting element into a receptacle defined by the drill bit, or by brazing the substrate of the cutting element directly into a preformed pocket, socket, or other receptacle formed in the drill bit. In one example, cutter pockets may be formed in the face of a matrix-type bit comprising tungsten carbide particles that are infiltrated or cast with a binder (e.g., a copper-based binder), as known in the art. Such drill bits are typically used for rock drilling, machining of wear resistant materials, and other operations which require high abrasion resistance or wear resistance. Generally, a rotary drill bit may include a plurality of polycrystalline abrasive cutting elements affixed to a drill bit body.

A PDC (as well as other superhard materials) may be fabricated by placing a layer of diamond crystals or grains adjacent one surface of a substrate and exposing the diamond grains and substrate to an ultra-high pressure and ultra-high temperature ("HPHT") process. Thus, a substrate and adjacent diamond crystal layer may be sintered under ultra-high temperature and ultra-high pressure conditions to cause the diamond crystals or grains to bond to one another. In addition, as known in the art, a catalyst may be employed for facilitating formation of polycrystalline diamond. In one example, a so-called "solvent catalyst" may be employed for facilitating the formation of polycrystalline diamond. For example, cobalt, nickel, and iron are among examples of solvent catalysts for forming polycrystalline diamond. In one configuration, during sintering, solvent catalyst from the substrate body (e.g., cobalt from a cobalt-cemented tungsten carbide substrate) becomes liquid and sweeps from the region behind the substrate surface next to the diamond powder and into the

diamond grains. Of course, a solvent catalyst may be mixed with the diamond powder prior to sintering, if desired.

Also, as known in the art, such a solvent catalyst may dissolve carbon at high temperatures. Such carbon may be dissolved from the diamond grains or portions of the diamond grains that graphitize due to the high temperatures of sintering. When the solvent catalyst is cooled, at least a portion of the carbon held in solution may precipitate or otherwise be expelled from the solvent catalyst and may facilitate formation of diamond bonds between adjacent or abutting diamond grains. Thus, the diamond grains become mutually bonded to form a polycrystalline diamond table upon the substrate. The solvent catalyst may remain in the diamond layer within the interstitial space between the diamond grains or the solvent catalyst may be at least partially removed and optionally replaced by another material, as known in the art. For instance, the solvent catalyst may be at least partially removed from the polycrystalline diamond by acid leaching. One example of a conventional process for forming polycrystalline diamond compacts is disclosed in U.S. Pat. No. 3,745,623 to Wentorf, Jr. et al., the disclosure of which is incorporated herein, in its entirety, by this reference.

Superhard materials (other than polycrystalline diamond) may also be formed by HPHT processing (i.e., sintering) or may be formed by other processes (e.g., chemical vapor deposition or any other suitable process), without limitation.

It may be appreciated that it would be advantageous to provide methods for forming superabrasive materials and apparatuses, structures, or articles of manufacture including such superabrasive material.

**SUMMARY**

One aspect of the instant disclosure relates to a superabrasive volume including a tungsten carbide layer. Such a superabrasive volume may comprise polycrystalline diamond, cubic boron nitride, diamond, silicon carbide, mixtures of the foregoing, or any composite including one or more of the foregoing materials and/or other superhard materials. Further, a tungsten carbide layer may be formed upon at least a portion of superabrasive volume. For example, a tungsten carbide layer may be formed upon at least a portion of a substantially planar surface and/or a side surface of the superabrasive volume. Optionally, such a superabrasive volume may be affixed to a substrate or to a drilling tool. For example, a superabrasive element/compact including tungsten carbide layer may be affixed to a drill bit or other drilling tool by brazing or any other suitable method.

Any of the aspects described in this application may be applicable to a polycrystalline diamond element or method of forming or manufacturing a polycrystalline diamond element.

Subterranean drill bits or other subterranean drilling or reaming tools including at least one of any superabrasive element encompassed by this application are also contemplated by the present invention.

Features from any of the above mentioned embodiments may be used in combination with one another, without limitation. In addition, other features and advantages of the instant disclosure will become apparent to those of ordinary skill in the art through consideration of the ensuing description, the accompanying drawings, and the appended claims.

**BRIEF DESCRIPTION OF THE DRAWINGS**

Further features of the subject matter of the instant disclosure, its nature, and various advantages will be more apparent

from the following detailed description and the accompanying drawings, which illustrate various exemplary embodiments, are representations, and are not necessarily drawn to scale, wherein:

FIG. 1A shows a perspective view of one embodiment of a superabrasive volume;

FIG. 1B shows a perspective view of a superabrasive element comprising the superabrasive volume shown in FIG. 1A including a tungsten carbide layer;

FIG. 2A shows a perspective view of another embodiment of a superabrasive volume;

FIG. 2B shows a side cross-sectional view of a superabrasive element comprising the superabrasive volume shown in FIG. 2A including a tungsten carbide layer;

FIG. 3 shows a schematic diagram of one embodiment of a method for forming a superabrasive compact encompassed by the present invention;

FIG. 4 shows a schematic diagram of an additional embodiment of a method for forming a superabrasive compact;

FIG. 5 shows a side cross-sectional view of one embodiment of a superabrasive compact encompassed by the present invention;

FIG. 6 shows a schematic diagram of a further embodiment of a method for forming a superabrasive compact;

FIG. 7 shows a side cross-sectional view of an additional embodiment of a superabrasive compact encompassed by the present invention;

FIG. 8 shows a side cross-sectional view of yet a further embodiment of a superabrasive compact encompassed by the present invention;

FIG. 9 shows a side cross-sectional view of an additional embodiment of a superabrasive element including a tungsten carbide layer encompassed by the present invention;

FIG. 10 shows a perspective view of a superabrasive compact encompassed by the present invention;

FIG. 11 shows a perspective view of another embodiment of a superabrasive element;

FIG. 12 shows a perspective view of a rotary drill bit including at least one superabrasive cutting element according to the present invention;

FIG. 13 shows a top elevation view of the rotary drill bit shown in FIG. 12;

FIG. 14A shows an enlarged side cross-sectional view of one embodiment of a rotatable cutting system including a tungsten carbide layer;

FIG. 14B shows an exploded, partial side cross-sectional view of the cutting element and cutting pocket shown in FIG. 14A; and

FIG. 15 shows a perspective view of an embodiment of an actuator assembly for applying torque to a rotatable cutting element, wherein at least one of the components includes a tungsten carbide layer.

#### DETAILED DESCRIPTION

The present invention relates generally to structures comprising at least one superabrasive material (e.g., diamond, boron nitride, silicon carbide, mixtures of the foregoing, or any material exhibiting a hardness exceeding a hardness of tungsten carbide) and methods of manufacturing such structures. Exemplary embodiments and features relating to the present invention are discussed hereinbelow.

The terms "superhard" and "superabrasive," as used herein, mean a material exhibiting a hardness exceeding a hardness of tungsten carbide. For example, polycrystalline diamond may be one embodiment of a superabrasive volume.

In another example, superabrasive material comprising a diamond-silicon carbide composite as disclosed in U.S. Pat. No. 7,060,641, the disclosure of which is incorporated herein, in its entirety, by this reference may be employed to form a superabrasive volume. More generally, cubic boron nitride, diamond, silicon carbide, or mixtures or any composite including one or more of the foregoing materials or other superhard materials may be employed.

More particularly, the present invention relates to a superabrasive mass or volume with a tungsten carbide layer. As used herein, the phrase "tungsten carbide layer" means a material substantially comprising tungsten carbide (which may be alloyed to a limited extent), wherein the tungsten carbide is not cemented or held in a binder or matrix. In one embodiment, a tungsten carbide layer may essentially consist of tungsten carbide or may consist entirely of tungsten carbide. Thus, explaining further, a tungsten carbide layer may be formed, for instance, by chemical vapor deposition, physical vapor deposition, chemical reactions, sintering (without a binder), or any suitable method. Accordingly, a cobalt-cemented tungsten carbide material or a tungsten carbide hard-facing (tungsten carbide particulate applied to a surface with a melted binder) material is not considered a tungsten carbide layer according to the above definition.

In one embodiment of a method of manufacturing a superabrasive element, a superabrasive volume including a tungsten carbide layer may be formed. Further, the superabrasive volume and a substrate may be bonded to one another. Such a method may be employed to form a superabrasive element with desirable characteristics. For instance, in one embodiment, such a process may allow for bonding of a so-called "thermally-stable" product ("TSP") or thermally-stable polycrystalline diamond ("TSD") or a partially thermally-stable (i.e., partially leached) polycrystalline diamond volume to a substrate to form a polycrystalline diamond element. In one embodiment, an HPHT process may be employed for bonding the polycrystalline diamond volume to the substrate. Such a polycrystalline diamond element may exhibit a desirable residual stress field and desirable thermal stability characteristics.

As described above, manufacturing sintered superabrasive materials, such as polycrystalline diamond involves the compression of superhard particles under extremely high pressure. Such compression may occur at room temperature, at least initially, and may result in the reduction of void space in the superhard particles due to brittle crushing, sliding, stacking, and/or otherwise consolidation. Thus, the superhard particles may sustain very high local pressures where they contact one another, but the pressures experienced on non-contacting surfaces of the superhard particles and in the interstitial voids may be, comparatively, low. Manufacturing superhard materials further involves heating the superhard particles. Such heating may increase the temperature of the superhard particles from room temperature to facilitate interparticle bonding (i.e., to a temperature and pressure where the desired superhard material is thermodynamically stable).

In the case of polycrystalline diamond, heating of diamond particles to at least to the melting point of a solvent catalyst is typically desired. Portions of the diamond particles under high local pressures may remain diamond, even at elevated temperatures. However, regions of the diamond particles that are not under high local pressure may begin to graphitize as temperature of such regions increases. Further, as a solvent-catalyst melts, it may infiltrate or "sweep" through the diamond particles. In addition, as known in the art, a solvent catalyst (e.g., cobalt, nickel, iron, etc.) may dissolve and transport carbon between the diamond grains and facilitate

diamond formation. Thus, the presence of solvent catalyst may facilitate the formation of diamond-to-diamond bonds in the sintered polycrystalline diamond material, resulting in formation of a coherent skeleton or matrix of bonded diamond particles or grains. Other types of catalysts besides metal solvent catalysts may be employed. For example, carbonate-based catalysts (e.g., magnesium carbonate ( $MgCO_3$ )), may be used to promote diamond-to-diamond bonds in the sintered polycrystalline diamond material.

One aspect of the present invention relates to a superabrasive volume including a tungsten carbide layer. More particularly, the present invention contemplates that one embodiment of a method of manufacturing a superabrasive compact may comprise forming a superabrasive volume including a tungsten carbide layer over at least a portion of an exterior surface of the superabrasive volume. In one embodiment, a tungsten carbide layer may be formed by chemical vapor deposition ("CVD") or variants thereof (e.g., plasma-enhanced CVD, etc., without limitation). Specifically, for example, one example of a commercially available CVD tungsten carbide layer (currently marketed under the trademark HARDIDE®) is currently available from Hardide Layers Inc. of Houston, Tex. In other embodiments, a tungsten carbide layer may be formed by physical vapor deposition ("PVD"), variants of PVD, high-velocity oxygen fuel ("HVOF") thermal spray processes, or any other suitable process, without limitation.

One of ordinary skill in the art will recognize that in some embodiments, the tungsten carbide layer may be formed prior to forming the superabrasive volume. For example, a tungsten carbide sheet or film may be positioned adjacent to a superabrasive powder (e.g., diamond powder, cubic boron nitride powder, silicon carbide powder, mixtures of the foregoing, etc.) and then the superabrasive powder may be sintered to form a superabrasive volume. In another example, a tungsten carbide layer may be initially formed and a superabrasive volume may be formed upon the tungsten carbide layer by CVD or any other suitable process.

More particularly, FIG. 1A shows a perspective view of one embodiment of a superabrasive volume **10**. As shown in FIG. 1A, in one embodiment, superabrasive volume **10** may be generally cylindrical and may include upper substantially planar surface **20**, side surface **22**, and lower substantially planar surface **24**. Further, as discussed above, superabrasive volume **10** may comprise polycrystalline diamond, cubic boron nitride, diamond, silicon carbide, mixtures of the foregoing, or any composite including one or more of the foregoing materials and/or other superhard materials. Additionally, a tungsten carbide layer may be formed upon at least a portion of superabrasive volume **10**. For example, FIG. 1B shows one embodiment of a superabrasive element **12** including a tungsten carbide layer **30** formed upon at least a portion of substantially planar surface **24**. Tungsten carbide layer **30** may exhibit a thickness of about 5  $\mu m$  to about 100  $\mu m$ , and more specifically about 5  $\mu m$  to about 60  $\mu m$ . Such a configuration may allow for superabrasive element **52** to be attached to a drilling tool or other apparatus. For example, superabrasive element **52** including tungsten carbide layer **30** may be affixed to a drill bit by brazing, since the tungsten carbide layer **30** may be wettable by a brazing alloy.

More generally, the present invention contemplates that tungsten carbide layer **30** may be formed upon any portion of substantially planar surface **24** and/or any portion of side surface **22** and/or any portion of substantially planar surface **20**, without limitation. Explaining further, any portion over which a tungsten carbide layer is not desired may be masked or otherwise precluded from forming the tungsten carbide

layer. In another embodiment, tungsten carbide may be formed over a selected region (e.g., the entire exterior or a portion thereof) of the superabrasive volume **10** and then selected portions of such tungsten carbide layer may be removed by grinding, electrical-discharge machining, chemical treatments, or any other suitable method, without limitation.

FIG. 2A shows another embodiment of a superabrasive volume **50** including an upper substantially planar surface **20**, 10 a side surface **22**, and a lower substantially planar surface **24**. As shown in FIG. 2A, superabrasive volume **50** may be substantially cylindrical, in one embodiment. Further, a tungsten carbide layer may be formed upon at least a portion of superabrasive volume **50**. For example, FIG. 2B shows one embodiment 15 of a superabrasive element **52** including a tungsten carbide layer **30** formed upon substantially planar surface **24** and over a majority of side surface **22**. Such a configuration may allow for superabrasive element **52** to be attached to a drilling tool or other apparatus. For example, superabrasive element **52** may be affixed to a drill bit by brazing, since the tungsten carbide layer **30** may be wet by a brazing alloy. More generally, the present invention contemplates that tungsten carbide layer **30** may be formed upon any portion of substantially planar surface **24** and/or any portion of side surface **22**, 20 and/or any portion of substantially planar surface **20**, without limitation. As described above, tungsten carbide layer **30** may be formed over a selected portion of superabrasive volume **30** via masking, selective removal, or any other suitable method.

One of ordinary skill in the art will understand that the 30 instant disclosure contemplates a tungsten carbide layer bonded to a superabrasive material. The instant disclosure contemplates that such a tungsten carbide layer may be bonded directly to a superabrasive material or one or more intermediary layer may extend between the superabrasive 35 material and the tungsten carbide layer. For example, an intermediary layer between the superabrasive material and the tungsten carbide layer may comprise tungsten, cobalt, molybdenum, tin, copper, or any metal, ceramic, or other selected material. Further, a tungsten carbide layer may 40 include other constituents, such as an alloying material or other element or compound. For example, tungsten carbide may be alloyed with fluorine. In another example, alternate layers of tungsten and tungsten carbide may be formed. Of course, additional layers of a selected material may be formed 45 upon a tungsten carbide layer, if desired.

Further, optionally, a method of manufacturing a superabrasive compact may further comprise affixing a superabrasive volume including a tungsten carbide layer to a substrate. For example, a superabrasive volume may be brazed, soldered, welded (including frictional or inertial welding), or otherwise affixed to a substrate. In another embodiment, the superabrasive volume may become affixed to a substrate by exposing the superabrasive volume and substrate to an elevated pressure (i.e., any pressure exceeding an ambient 50 atmospheric pressure; e.g., exceeding about 20 kilobar, at least about 60 kilobar, or between about 20 kilobar and about 60 kilobar) and an elevated temperature (e.g., at least about 60 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 94

a temperature of at least about 1000° Celsius. In one example, a pressure of at least about 60 kilobar may be developed. Regarding temperature, in one example, a temperature of at least about 1,350° Celsius may be developed. Further, such an HPHT process may cause the superabrasive element to become affixed to the substrate. Optionally, a braze material may be provided to ultimately extend between and affix the superabrasive element and the substrate to one another. Such a braze material may be at least partially melted to affix the superabrasive element to the substrate upon cooling of the braze material.

One aspect of the present invention relates to a manufacturing method for forming a superabrasive compact. Generally, a manufacturing method for forming a superabrasive compact may include forming a superabrasive element comprising a superabrasive volume and a tungsten carbide layer. Further, the superabrasive element may be affixed to a substrate. FIG. 3 shows a schematic diagram of a method 32 for forming a superabrasive compact. As shown in FIG. 3, method 32 comprises process action 34 and process action 36. Particularly, as shown in FIG. 3, a superabrasive element may be provided (as represented by process action 34 in FIG. 3) by forming superabrasive volume including a tungsten carbide layer. Further, the superabrasive element may be affixed to a substrate (as represented by process action 36 in FIG. 3) to form a superabrasive compact.

For example, a superabrasive element comprising a superabrasive volume including a tungsten carbide layer may be positioned adjacent to a substrate and the assembly may be exposed to an HPHT process. Optionally, during the HPHT process, at least one constituent (e.g., a metal) of the substrate and/or the superabrasive element may at least partially melt. Further, upon cooling, the superabrasive element may be affixed to the substrate. Optionally, such an HPHT process may generate a beneficial residual stress field within each of the superabrasive volume and the substrate. Explaining further, a coefficient of thermal expansion of a superabrasive material may be substantially less than a coefficient of expansion of a substrate. In one example, a superabrasive volume may comprise polycrystalline diamond and a substrate may comprise cobalt-cemented tungsten carbide. The present invention contemplates that selectively controlling the temperature and/or pressure during an HPHT process may allow for selectively tailoring a residual stress field developed within a superabrasive volume and/or a substrate to which the superabrasive volume is affixed. Furthermore, the presence of a residual stress field developed within the superabrasive and/or the substrate may be beneficial.

FIG. 4 shows a schematic diagram representing another embodiment of a method 38 for forming a superabrasive compact, the method comprising a process action 42 and a process action 46. As shown in FIG. 4, process action 42 may include forming a superabrasive element comprising a superabrasive volume and a tungsten carbide layer. In addition, as represented by process action 44, the superabrasive element may be positioned adjacent to a substrate. Further, at least one constituent of the superabrasive element, the substrate, or both may be at least partially melted (as represented by process action 46). At least partially melting of such at least one constituent may cause the superabrasive element to be affixed or bonded to the substrate. Such a method 38 may be relatively effective for bonding a superabrasive element to a substrate.

Explaining further, at least one constituent of a substrate, at least one constituent of a superabrasive volume or a combination of the foregoing may be employed to affix the superabrasive volume to the substrate. In one embodiment, a supera-

brasive volume may comprise a sintered structure formed by a previous HPHT process. For example, a superabrasive volume may comprise a polycrystalline diamond structure (e.g., a diamond table) or any other sintered superabrasive material, without limitation. In other embodiments, superabrasive volume may comprise boron nitride, silicon carbide, fullerenes, or a material having a hardness exceeding a hardness of tungsten carbide, without limitation. In one example, a substrate may comprise a cobalt-cemented tungsten carbide. Accordingly, at elevated temperatures and pressures, such cobalt may at least partially melt and/or infiltrate or wet the superabrasive volume. Upon solidification of the cobalt, the substrate and the superabrasive volume may be affixed to one another.

FIG. 5 shows a side cross-sectional view of a superabrasive compact 40 comprising a superabrasive element 12, as described herein, bonded to a substrate 110. In one embodiment, superabrasive volume 10 may comprise polycrystalline diamond and a tungsten carbide layer 30, and substrate 110 may comprise a cobalt-cemented tungsten carbide. The present invention further contemplates that if superabrasive volume 10 comprises polycrystalline diamond, a catalyst (e.g., cobalt) used to form the superabrasive volume 10 may be at least partially removed from the polycrystalline diamond. For example, a catalyst (e.g., cobalt) may be at least partially removed from polycrystalline diamond by exposing the polycrystalline diamond to an acid, exposing the polycrystalline diamond to an electrolytic processes, combinations of the foregoing, or any other suitable method.

Another aspect of the present invention relates to bonding or affixing a superabrasive volume to a substrate by at least partially melting a braze material. For example, FIG. 6 shows a further embodiment of a manufacturing method 48 for forming a superabrasive element, the method comprising a process action 54, process action 56, and process action 58. As shown in FIG. 6, process action 54 may include forming a superabrasive element comprising a superabrasive volume and a tungsten carbide layer. Further, as represented by process action 56, the superabrasive element and, as represented by process action 58, the superabrasive element may be brazed to the substrate.

Exemplary braze, in one example, may be referred to as "Group Ib solvents" (e.g., copper, silver, and gold) and may optionally contain one or more carbide former (e.g., titanium, vanadium, chromium, manganese, zirconium, niobium, molybdenum, technetium, hafnium, tantalum, tungsten, or rhenium, without limitation). Accordingly, exemplary compositions may include gold-tantalum Au-Ta, silver-copper-titanium (Ag—Cu—Ti), or any mixture of any Group Ib solvent(s) and, optionally, one or more carbide former. Other suitable braze materials may include a metal from Group VIII in the periodic table, (e.g., iron, cobalt, and nickel). In one embodiment, a braze material may comprise an alloy of about 4.5% titanium, about 26.7% copper, and about 68.8% silver, otherwise known as TICUSIL®, which is currently commercially available from Wesgo Metals, Hayward, Calif. In a further embodiment, a braze material may comprise an alloy of about 25% silver, about 37% copper, about 10% nickel, about 15% palladium, and about 13% manganese, otherwise known as PALNICUROM® 10, which is also currently commercially available from Wesgo Metals, Hayward, Calif. In an additional embodiment, a braze material may comprise an alloy of about 64% iron and about 36% nickel, commonly referred to as Invar. In again a further embodiment, a braze material may comprise a single metal such as for example, cobalt. One of ordinary skill in the art will understand that brazing may be performed in an inert environment (i.e., an

environment that inhibits oxidation), which may be a beneficial environment for proper functioning of the braze alloy.

Optionally, a superabrasive volume and at least a portion of a substrate may be sealed within an enclosure under vacuum or an inert atmosphere (e.g., at least substantially surrounded by an inert gas, such as argon, nitrogen, and/or helium, without limitation). Generally, any methods or systems may be employed for sealing, under vacuum or inert atmosphere, a superabrasive volume or element and at least a portion of a substrate within an enclosure. For example, U.S. Pat. No. 4,333,902 to Hara, the disclosure of which is incorporated, in its entirety, by this reference, and U.S. patent application Ser. No. 10/654,512 to Hall, et al., filed 3 Sep. 2003 the disclosure of which is incorporated, in its entirety, by this reference, each disclose methods and systems related to sealing an enclosure under vacuum or inert atmosphere. U.S. patent application Ser. No. 11/545,929, the disclosure of which is incorporated, in its entirety, by this reference also discloses another example of methods and systems for sealing an enclosure in an inert environment.

Accordingly, generally, the present invention contemplates a braze material may be at least partially melted to affix the substrate to the superabrasive element. Subsequent cooling of the braze material may cause solidification of the braze material, and affixation of the superabrasive element to the substrate via the braze material. In one example, a superabrasive element, a braze material, and a substrate may be exposed to an HPHT process. Such an HPHT process may cause the superabrasive element to be affixed to the substrate via the braze material. In another embodiment, a braze material, substrate, and/or superabrasive element may be heated to effect affixation of the superabrasive element and the substrate.

In another example, a superabrasive element, a braze material, and a substrate may be exposed to a pressure exceeding an ambient atmospheric pressure (e.g., at least about 60 kilobar). Further, the braze material may be at least partially melted. Optionally, the braze material may be at least partially melted while the elevated pressure is applied to the enclosure. In one embodiment, a braze material may exhibit a melting temperature of at least about 900° Celsius. For example, in one embodiment, a braze material may exhibit a melting temperature of about 900° Celsius in the case of TICUSIL®. In another embodiment, a braze material may exhibit a melting temperature of about 1013° Celsius in the case of PALNI-CUROM® 10. In a further embodiment, a braze material may exhibit a melting temperature of about 1427° Celsius in the case of Invar. In yet a further embodiment, a braze material may exhibit a melting temperature of about 1493° Celsius in the case of cobalt. One of ordinary skill in the art will understand that the actual melting temperature of a braze material is dependent on the pressure applied to the braze material and the composition of the braze material. Accordingly, the values listed above are merely for reference. In addition, the braze material may be at least partially solidified while the enclosure is exposed to the selected, elevated pressure (e.g., exceeding about 20 kilobar, at least about 60 kilobar, or between about 20 kilobar and about 60 kilobar). Such a process may affix or bond the superabrasive element to the substrate. Moreover, solidifying the braze material while the enclosure is exposed to an elevated pressure exceeding an ambient atmospheric pressure may develop a selected level of residual stress within the superabrasive element upon cooling to ambient temperatures and upon release of the elevated pressure.

The present invention contemplates that an article of manufacture comprising a superabrasive volume may be manufac-

tured by performing the above-described processes or variants thereof. In one example, apparatuses including polycrystalline diamond may be useful for cutting elements, heat sinks, wire dies, and bearing apparatuses, without limitation. Optionally, a superabrasive volume may comprise polycrystalline diamond. Thus, a polycrystalline diamond volume may be formed by any suitable process, without limitation. Optionally, such a polycrystalline diamond volume may comprise so-called "thermally stable" polycrystalline diamond material. For example, a catalyst material (e.g., cobalt, nickel, iron, or any other catalyst material), which may be used to initially form the polycrystalline diamond volume, may be at least partially removed (e.g., by acid leaching or as otherwise known in the art) from the polycrystalline diamond volume. In one embodiment, a polycrystalline diamond volume that is substantially free of a catalyzing material may be affixed or bonded to a substrate. Such a polycrystalline diamond apparatus may exhibit desirable wear characteristics. In addition, as described above, such a polycrystalline diamond apparatus may exhibit a selected residual stress field that is developed within the polycrystalline diamond volume and/or the substrate.

In a specific example, a polycrystalline diamond element comprising a polycrystalline diamond volume and a tungsten carbide layer may be affixed to a substrate by a braze material. In one example, the polycrystalline diamond element, braze material, and substrate may be exposed to an HPHT process. Such an HPHT process may cause the polycrystalline diamond element to be affixed to the substrate via the braze material, as described above. Furthermore, a polycrystalline diamond element so formed may exhibit the beneficial residual stress characteristics described above. For example, a polycrystalline diamond element, a substrate, and a braze material may be exposed to a pressure exceeding an ambient atmospheric pressure (e.g., exceeding about 20 kilobar, at least about 60 kilobar, or between about 20 kilobar and about 60 kilobar). Further, the braze material may be at least partially melted. Of course, the braze material may be at least partially melted during exposure of the enclosure to an elevated pressure, prior to such exposure, after such exposure, or any combination of the foregoing. In addition, the braze material may be solidified while the enclosure is exposed to a selected, elevated pressure (e.g., exceeding about 20 kilobar, at least about 60 kilobar, or between about 20 kilobar and about 60 kilobar). In other embodiments, the braze material may be solidified prior to such exposure, after such exposure, or any combination of the foregoing. Such a process may affix or bond the preformed polycrystalline diamond element to the substrate. Moreover, solidifying the braze material while the enclosure is exposed to an elevated pressure may develop a selected level of residual stress within the polycrystalline diamond element (i.e., the polycrystalline diamond volume, the braze material, and/or the substrate) upon cooling to ambient temperatures and upon release of the elevated pressure.

Thus, as explained above, a superabrasive compact may be formed by any process encompassed by the present invention. FIG. 7 shows a schematic, side cross-sectional view of a superabrasive compact 41 including a superabrasive element 12 (comprising superabrasive volume 10 and tungsten carbide layer 30, which is depicted as a line, for clarity), a substrate 110, and braze material 60. As shown in FIG. 7, braze material 60 may be positioned between the superabrasive element 12 and the substrate 20.

In another embodiment, a plurality of superabrasive volumes may be affixed to one another. For example, FIG. 8 shows a schematic, side cross-sectional view of a superabra-

## 11

sive compact **43**. As shown in FIG. 8, superabrasive compact **43** comprises a first superabrasive element **12** and a superabrasive volume **55**. In one embodiment, a superabrasive volume **55** (e.g., a polycrystalline diamond table) may be formed upon the substrate **110** in an HPHT process. In other embodiments, superabrasive volume **55** may include a tungsten carbide layer and may be affixed to substrate **110** according to the present invention, if desired. As shown in FIG. 8, a braze material **60** may be positioned between superabrasive element **12** (comprising superabrasive volume **10** and tungsten carbide layer **30**) and superabrasive volume **55**. In a further embodiment, a comparatively thin superabrasive volume may be affixed to a comparatively thicker superabrasive volume. For example, FIG. 9 shows a schematic, side cross-sectional view of a superabrasive element **45**. As shown in FIG. 9, superabrasive element **45** comprises a first superabrasive volume **10** and a second superabrasive volume **50**. As shown in FIG. 9, a braze material **60** may be positioned between superabrasive volume **10** and superabrasive volume **50**. Further, superabrasive volume **50** may include a tungsten carbide layer **30**. Thus, superabrasive element **52** (comprising superabrasive volume **50** and tungsten carbide layer **30**) may be affixed to superabrasive volume **10**.

One of ordinary skill in the art will appreciate from the foregoing exemplary embodiments that many variations and/or configurations (e.g., three or more superabrasive volumes bonded to one another, respectively) for superabrasive structures including a plurality of superabrasive volumes are contemplated by the present invention. More specifically, one of ordinary skill in the art will appreciate that a plurality of superabrasive volumes may be bonded to one another (and, optionally, to a superabrasive compact or other substrate) by appropriately positioning (e.g., stacking) each of the plurality of superabrasive volumes and exposing the enclosure to an increased temperature and/or an elevated pressure, brazing or any suitable method, without limitation. Optionally, at least one superabrasive volume and one or more layers of superabrasive particulate (i.e., powder) may be exposed to elevated pressure and temperature sufficient to sinter the superabrasive particulate and form at least one superabrasive volume.

In one application, the present invention contemplates that a superabrasive volume/element may be affixed to a drilling structure, such as a drill bit. For example, FIG. 10 shows a perspective view of a superabrasive compact **40**, **41**, and **43**. As shown in FIG. 10, substrate **110** may be substantially cylindrical and superabrasive volume **10** may also be substantially cylindrical. As shown in FIG. 10, substrate **110** and superabrasive element **12** may be bonded to one another along an interface **33**. Such an interface **33** is defined between substrate **110** and superabrasive element **12** and may exhibit a selected non-planar topography, if desired, without limitation. Further, optionally, a braze material may be positioned between substrate **110** and superabrasive element **12**, as discussed above.

Further, a selected superabrasive table edge geometry **31** may be formed upon superabrasive element **12** prior to bonding to substrate **110** or subsequent to bonding of the superabrasive element **12** to the substrate **110**. For example, edge geometry **31** may comprise a chamfer, buttress, any other edge geometry, or combinations of the foregoing and may be formed by grinding, electrical-discharge machining, or by other machining or shaping processes. Also, a substrate edge geometry **23** may be formed upon substrate **110** by any machining process or by any other suitable process. Further, such substrate edge geometry **23** may be formed prior to or subsequent to bonding of the superabrasive element **12** to the substrate **110**, without limitation. Of course, in one embodiment, the present invention contemplates that superabrasive element **12** may comprise a polycrystalline diamond volume and may be affixed to a substrate **110** comprising a cobalt-cemented tungsten carbide substrate to form a polycrystalline diamond element. For example, such a polycrystalline diamond element may be useful for, for example, cutting processes or bearing surface applications, among other applications.

## 12

In another embodiment, a superabrasive element may be configured to be affixed to a drilling structure. For example, FIG. 11 shows a perspective view of a superabrasive element **45**, **52**, as described above. As shown in FIG. 11, superabrasive element **45**, **52** may be substantially cylindrical. As also shown in FIG. 11, superabrasive element **45**, **52** may include tungsten carbide layer **30**. Further, a selected superabrasive table edge geometry **31** may be formed upon superabrasive element volume **10**, **50**, if desired. For example, edge geometry **31** may comprise a chamfer, buttress, any other edge geometry, or combinations of the foregoing and may be formed by grinding, electrical-discharge machining, or by other machining or shaping processes. Also, edge geometry **123** may be formed upon substrate **110** prior to forming tungsten carbide layer **30** or subsequent to forming tungsten carbide layer **30**. Such edge geometry **123** may be formed by any machining process or by any other suitable process. Of course, in one embodiment, the present invention contemplates that superabrasive volume **10**, **50** may comprise a polycrystalline diamond volume. Such a polycrystalline diamond element may be useful for, for example, cutting processes or bearing surface applications, among other applications.

The present invention also contemplates that the method and apparatuses discussed above may employ polycrystalline diamond that is initially formed with a catalyst and from which such catalyst is at least partially removed. Explaining further, in one example, during sintering of diamond powder, a catalyst material (e.g., cobalt, nickel, etc.) may be employed for facilitating formation of polycrystalline diamond. More particularly, diamond powder placed adjacent to a cobalt-cemented tungsten carbide substrate and subjected to an HPHT sintering process may wick or sweep molten cobalt into the diamond powder. In other embodiments, catalyst may be provided within the diamond powder, as a layer of material between the substrate and diamond powder, or as otherwise known in the art. In either case, such catalyst (e.g., cobalt) may remain in the polycrystalline diamond table upon sintering and cooling. As also known in the art, such a catalyst material may be at least partially removed (e.g., by acid-leaching or as otherwise known in the art) from at least a portion of the volume of polycrystalline diamond (e.g., a table) formed upon a substrate or otherwise formed. In one embodiment, catalyst removal may be substantially complete to a selected depth from an exterior surface of the polycrystalline diamond table, if desired, without limitation. Such catalyst removal may provide a polycrystalline diamond material with increased thermal stability, which may also beneficially affect the wear resistance of the polycrystalline diamond material.

More particularly, relative to the above-discussed methods and superabrasive elements, the present invention contemplates that a superabrasive volume may be at least partially depleted of catalyst material. In one embodiment, a superabrasive volume may be at least partially depleted of a catalyst material prior to bonding to a substrate. In another embodiment, a superabrasive volume may be bonded to a substrate by any of the methods (or variants thereof) discussed above and, subsequently, a catalyst material may be at least partially removed from the superabrasive volume. In either case, for

example, a preformed polycrystalline diamond volume may initially include cobalt that may be subsequently at least partially removed (optionally, substantially all of the cobalt may be removed) from the polycrystalline diamond volume (e.g., by an acid leaching process or any other process, without limitation).

One of ordinary skill in the art will understand that superabrasive materials, compacts, and/or elements may be utilized in many applications. For instance, wire dies, bearings, artificial joints, inserts, cutting elements, and heat sinks may include polycrystalline diamond. Thus, the present invention contemplates that any of the methods encompassed by the above-discussion related to forming superabrasive element may be employed for forming an article of manufacture comprising polycrystalline diamond. As mentioned above, in one example, an article of manufacture may comprise polycrystalline diamond. In one embodiment, the present invention contemplates that a volume of polycrystalline diamond may be affixed to a substrate.

Some examples of articles of manufacture comprising polycrystalline diamond are disclosed by, inter alia, U.S. Pat. Nos. 4,811,801, 4,268,276, 4,410,054, 4,468,138, 4,560,014, 4,738,322, 4,913,247, 5,016,718, 5,092,687, 5,120,327, 5,135,061, 5,154,245, 5,364,192, 5,368,398, 5,460,233, 5,480,233, 5,544,713, and 6,793,681. Thus, the present invention contemplates that any process encompassed herein may be employed for forming superabrasive elements/compacts (e.g., "PDC cutters" or polycrystalline diamond wear elements) for such apparatuses or the like.

As may be appreciated from the foregoing discussion, the present invention further contemplates that at least one superabrasive element/compact as described above may be affixed or coupled to a rotary drill bit for subterranean drilling. Such a configuration may provide a cutting element with enhanced properties in comparison to a conventionally formed cutting element. For example, FIGS. 12 and 13 show a perspective view and a top elevation view, respectively, of an example of an exemplary rotary drill bit 301 of the present invention including at least one superabrasive compact/element 40, 41, 43, 45, or 52 secured the bit body 321 of rotary drill bit 301 (e.g., by brazing or by any suitable affixation structure or method). Such superabrasive compact/element 40, 41, 43, 45, or 52 may be manufactured according to the above-described processes of the present invention, may exhibit structural characteristics as described above, or both.

Referring to FIGS. 12 and 13, generally, rotary drill bit 301 includes a bit body 321 which defines a leading end structure for drilling into a subterranean formation by rotation about longitudinal axis 311 and application of weight-on-bit. More particularly, rotary drill bit 301 may include radially and longitudinally extending blades 310 including leading faces 334. Further, circumferentially adjacent blades 310 define so-called junk slots 338 therebetween. As shown in FIGS. 12 and 13, rotary drill bit 301 may also include, optionally, superabrasive cutting elements 308 (e.g., generally cylindrical cutting elements such as PDC cutters) which may be a superabrasive element/compact according to the present invention or which may be conventional, without limitation. Additionally, rotary drill bit 301 includes nozzle cavities 318 for communicating drilling fluid from the interior of the rotary drill bit 301 to the superabrasive cutting elements 308, face 339, and threaded pin connection 360 for connecting the rotary drill bit 301 to a drilling string, as known in the art.

It should be understood that although rotary drill bit 301 includes at least one compact/element 40, 41, 43, 45, or 52, the present invention is not limited by such an example. Rather, a rotary drill bit according to the present invention

may include, without limitation, one or more cutting elements according to the present invention. Optionally, each of the compact/element 40, 41, 43, 45, 308, or 52 shown in FIGS. 12 and 13 may be formed according to processes contemplated by the present invention. Also, it should be understood that FIGS. 12 and 13 merely depict one example of a rotary drill bit employing at least one cutting element of the present invention, without limitation. More generally, the present invention contemplates that drill bit 301 may represent any 10 number of earth-boring tools or drilling tools, including, for example, core bits, roller-cone bits, fixed-cutter bits, eccentric bits, bicenter bits, reamers, reamer wings, or any other downhole tool including polycrystalline diamond cutting elements or inserts, without limitation.

15 The present invention further contemplates that a tungsten carbide layer may be beneficial for structures disclosed in U.S. application Ser. No. 11/247,574, entitled "Cutting element apparatuses, drill bits including same, methods of cutting, and methods of rotating a cutting element," the disclosure of which is incorporated, in its entirety, by this reference. For example, FIG. 14A shows an enlarged cross-sectional view of an embodiment of an actuator assembly 240 for applying torque to a rotatable cutting element. Actuator assembly 240 generally represents a device capable of transforming electricity or hydraulic energy generated and supplied by power source 230 into torque for rotating cutting element 270. In at least one embodiment, actuator assembly 240 comprises a motor (e.g., an electric motor or a hydraulic motor) that converts the electricity or hydraulic energy generated and supplied by power source 230 into torque. For example, FIG. 14A shows an actuator assembly 240 comprising a relatively compact motor (such as, for example, an electrically-powered geared motor or stepper motor) configured to generate and apply torque to a drive shaft 276 coupled to a substrate 272 of cutting element 270. Optionally, the torque and speed of rotation of drive shaft 276 relative to the torque and speed of rotation generated by actuator assembly 240 may be controlled by a transmission 255 coupled to actuator assembly 240. Generally, transmission 255 may represent a gearbox or other device and may be desirable for converting an unsuitably high speed and low torque generated by an actuator assembly 240 (e.g., an electrically-powered motor) to a lower speed with higher torque, or vice versa.

As shown in FIG. 14A, actuator assembly 240 may be 45 housed within recess 260 defined within a blade 212 of a drill bit. Also, optionally, a biasing element 190 (e.g., a Belleville washer spring, a coil spring, etc.) may be positioned between the actuator assembly 240 and the bit body (e.g., bit blade 212) so that cutting element 270 is biased toward cutting pocket 215. Recess 260 may, optionally, be sealed and pressurized to protect actuator 240 from excessive exposure to drilling fluids. Cutting element 270 generally represents any 50 form of cutting structure (e.g., a superabrasive compact/element encompassed by the present invention) capable of cutting a subterranean formation. In addition, drive shaft 276 may be mechanically coupled to substrate 272 of cutting element. Also, cutting element 270 may be rotatably mounted within a cutting pocket 215 defined in bit blade 212 of a drill bit. Cutting pocket 215 of bit blade 212 may be generally 55 configured similar to cutting pocket 115 to surround at least a portion of a periphery of cutting element 270 when positioned within cutting pocket 215. In addition, optionally, a separation element 165 (e.g., a washer element or the like) may be positioned between front surface of cutting pocket 215 and a back surface 275 of substrate 272 of cutting element 270.

In general, the present invention contemplates that at least one of the cutting element 270 and the cutting pocket 215 may

## 15

include a tungsten carbide layer. Optionally, both of the cutting element and the cutting pocket 215 may include a tungsten carbide layer. In one embodiment, a tungsten carbide layer may be formed upon at least a portion of a side surface 273 or back surface 275 of the cutting element 270 adjacent to cutting pocket 215. More particularly, FIG. 14B shows an exploded, partial, side cross-sectional view of cutting element 215 and cutting pocket 215. As shown in FIG. 14B, cutting element 270 may include a tungsten carbide layer 299A, a tungsten carbide layer 299B, or both. One of ordinary skill in the art will understand that any portion of side surface 273, back surface 275, or both (e.g., a continuous tungsten carbide layer formed over at least a portion of side surface 273 and at least a portion of back surface 275) may include a tungsten carbide layer, without limitation. Further, as shown in FIG. 14B, cutting pocket 215 may include a tungsten carbide layer 299C, a tungsten carbide layer 299D, or both. One of ordinary skill in the art will understand that any portion of side surface 217, back surface 219, or both (e.g., a continuous tungsten carbide layer formed over at least a portion of side surface 217 and at least a portion of back surface 219) may include a tungsten carbide layer, without limitation. Such a configuration (i.e., a tungsten carbide layer formed upon at least one of: a cutting element and a cutting pocket) may inhibit wear and/or friction between the cutting element 270 and the cutting pocket 215. However, the present invention contemplates that a tungsten carbide layer formed upon at least a portion of a cutting structure, a cutting pocket, or both may be beneficial to both rotating cutting elements and non-rotating cutting elements, without limitation.

In another embodiment, FIG. 15 shows a push rod 187 configured for interacting with engaging features 188 formed into a substrate 172 to rotate cutting element 170. More particularly, an end 189 of push rod 187 may be structured for interacting with engaging features 188 (e.g., a surface or other aspect of a recess) to rotate cutting element 170. Thus, it may be understood that an actuator assembly may cause push rod 187 to reciprocate (i.e., toward and away from) with respect to substrate 172. The present invention generally contemplates that at least a portion of push rod 187 and/or cutting element 170 may include a tungsten carbide layer. Particularly, in one embodiment, region 199 of push rod 187 may include a tungsten carbide layer 399. Further, as shown in FIG. 15, cutting element 170 may include a tungsten carbide layer 299A, a tungsten carbide layer 299B, or both. One of ordinary skill in the art will understand that any portion of side surface 173, back surface 175, or both (e.g., a continuous tungsten carbide layer formed over at least a portion of side surface 173 and at least a portion of back surface 175) may include a tungsten carbide layer, without limitation.

While certain embodiments and details have been included herein and in the attached invention disclosure for purposes of illustrating the invention, it will be apparent to those skilled in the art that various changes in the methods and apparatus disclosed herein may be made without departing from the scope of the invention, which is defined in the appended claims. The words "including" and "having," as used herein, including the claims, shall have the same meaning as the word "comprising."

The invention claimed is:

1. A rotary drill bit, comprising:  
a bit body configured to engage a subterranean formation during drilling; and  
a plurality of polycrystalline diamond cutting elements mounted to the bit body, at least one of the plurality of polycrystalline diamond cutting elements including:

## 16

a sintered polycrystalline diamond body including an upper surface, a back surface, and at least one side surface extending therebetween; and

a chemically-vapor-deposited tungsten carbide layer attached to the back surface and a majority of the at least one side surface of the sintered polycrystalline diamond body, the chemically-vapor-deposited tungsten carbide layer exhibiting a thickness of about 5  $\mu\text{m}$  to about 100  $\mu\text{m}$ , the chemically-vapor-deposited tungsten carbide layer further attached to the bit body.

2. The rotary drill bit of claim 1 wherein the thickness of the chemically-vapor-deposited tungsten carbide layer is about 5  $\mu\text{m}$  to about 60  $\mu\text{m}$ .

3. The rotary drill bit of claim 1 wherein the chemically-vapor-deposited tungsten carbide layer consists essentially of tungsten carbide.

4. The rotary drill bit of claim 1 wherein the chemically-vapor-deposited tungsten carbide layer comprises fluorine.

5. The rotary drill bit of claim 1 wherein the chemically-vapor-deposited tungsten carbide layer covers a substantial portion of the at least one side surface of the sintered polycrystalline diamond body.

6. The rotary drill bit of claim 1 wherein the sintered polycrystalline diamond body comprises thermally-stable polycrystalline diamond.

7. The rotary drill bit of claim 1, further comprising a braze material bonding the chemically-vapor-deposited tungsten carbide layer to the bit body.

8. The rotary drill bit of claim 7 wherein the braze material comprises a silver-copper braze material.

9. The rotary drill bit of claim 7 wherein the braze material comprises an iron-nickel braze material.

10. The rotary drill bit of claim 1 wherein the at least one of the plurality of polycrystalline diamond cutting elements comprises a substrate bonded to the bit body and the chemically-vapor-deposited tungsten carbide layer.

11. The rotary drill bit of claim 10 wherein the substrate comprises a cemented carbide substrate.

12. A rotary drill bit, comprising:  
a bit body configured to engage a subterranean formation during drilling; and

a plurality of polycrystalline diamond cutting elements mounted to the bit body, at least one of the plurality of polycrystalline diamond cutting elements including:  
a thermally-stable polycrystalline diamond body including an upper surface, a back surface, and at least one side surface extending therebetween; and  
a tungsten carbide layer attached to the back surface and a majority of the at least one side surface of the thermally-stable polycrystalline diamond body and to the bit body, the tungsten carbide layer exhibiting a thickness of about 5  $\mu\text{m}$  to about 100  $\mu\text{m}$ .

13. The rotary drill bit of claim 12 wherein the thickness of the tungsten carbide layer is about 5  $\mu\text{m}$  to about 60  $\mu\text{m}$ .

14. The rotary drill bit of claim 12 wherein the tungsten carbide layer covers a substantial portion of the at least one side surface of the thermally-stable polycrystalline diamond body.

15. The rotary drill bit of claim 12 wherein the tungsten carbide layer comprises a chemically-vapor-deposited tungsten carbide layer.

16. A rotary drill bit, comprising:  
a bit body configured to engage a subterranean formation during drilling; and

**17**

a plurality of polycrystalline diamond cutting elements mounted to the bit body, at least one of the plurality of polycrystalline diamond cutting elements consisting essentially of:

a sintered polycrystalline diamond body including an upper surface, a back surface, and at least one side surface extending therebetween; and

a tungsten carbide layer attached to the back surface of the polycrystalline diamond body and brazed to the bit body.

**17.** The rotary drill bit of claim **16** wherein the tungsten carbide layer exhibits a thickness of about 5  $\mu\text{m}$  to about 100  $\mu\text{m}$ .

**18.** The rotary drill bit of claim **16** wherein the tungsten carbide layer exhibits a thickness of about 5  $\mu\text{m}$  to about 60  $\mu\text{m}$ .

**19.** The rotary drill bit of claim **16** wherein the tungsten carbide layer consists essentially of tungsten carbide.

**20.** The rotary drill bit of claim **16** wherein the tungsten carbide layer covers a substantial portion of the at least one side surface of the sintered polycrystalline diamond body.

**18**

**21.** The rotary drill bit of claim **16** wherein the sintered polycrystalline diamond body comprises thermally-stable polycrystalline diamond.

**22.** A method of manufacturing a rotary drill bit, comprising:

providing a polycrystalline diamond cutting element consisting essentially of:

a sintered polycrystalline diamond body including an upper surface, a back surface, and at least one side surface extending therebetween; and

a tungsten carbide layer attached to the back surface of the polycrystalline diamond body; and

brazing the tungsten carbide layer of the polycrystalline diamond cutting element directly to a bit body of the rotary drill bit.

**23.** The method of claim **22** wherein the tungsten carbide layer covers a majority of the at least one side surface of the sintered polycrystalline diamond body.

**24.** The method of claim **22** wherein the tungsten carbide layer comprises a chemically-vapor-deposited tungsten carbide layer.

\* \* \* \* \*